

## UNITED STATES PATENT OFFICE

2,426,254

ANODIC TREATMENT OF MAGNESIUM AND  
ITS ALLOYS TO FORM PROTECTIVE  
COATINGS THEREONHerbert Waterman, Los Angeles, Calif., assignor  
to Turco Products, Inc., Los Angeles, Calif., a  
corporation of CaliforniaNo Drawing. Application April 23, 1943,  
Serial No. 484,218

9 Claims. (Cl. 204—56)

1

This invention has to do with the formation of protective coatings on magnesium and magnesium alloys by electrolytic treatment and relates more particularly to anodic treatment and electrolytic baths for the purpose.

Although magnesium and its alloys have become increasingly recognized in recent years as having peculiar advantages in industry, a difficulty in their use has been the lack of suitable methods of providing a really dependable protective coating on the surface of the metal to safeguard against corrosion and to provide a permanent base for paint. Many such methods were proposed which may be classified under three headings: paint applications directly over the metal surface, chemical dip treatments, and electrochemical treatments, or combinations of those methods. A chemical dip treatment followed by an application of a paint coating has been deemed the best procedure heretofore.

The service performance of surface protection of magnesium and its alloys provided by such methods has been erratic and unreliable, and has left much to be desired. They provide no way to tell in advance whether any coating on any particular piece of magnesium or its alloy will perform adequately in service. The widespread use of magnesium in the aeroplane and other industries is retarded to a large extent by this uncertainty.

According to the present practices in this art there is no certainty that the coated magnesium article possesses a really dependable coating, and there is no reliable method of determining from the coating operation whether the article is of proper quality, or whether it contains segregation of alloying constituents or whether the surface area contains foreign elements which will render the coating poor. Thus, in the past, many failures of the coated material have resulted which have been inexplicable.

By my invention I aim to overcome those past uncertainties and shortcomings, particularly insofar as electrochemical treatment is concerned, and to provide a method of and electrolyte for electrolytic treatment of magnesium and its alloys which is controllable, fully dependable, enables uniform and simplified shop practices to produce coatings of definitely determinable character, and which does not require any elaborate control facilities.

Another object is the production of a dense coating which is self sealing so that, upon its completion, it will provide an adequate protection for the surface of magnesium and its alloys.

2

Another object is the provision of an improved electrochemical bath in which the coating is produced.

Still further objects and corresponding advantages are inherent in my invention and those will appear obvious from the following detailed explanation of the presently preferred procedure.

In a preferred practice of my invention I use an electrolyte made up of a solution of soluble carbonate, using relatively pure sodium carbonate in quantities sufficient to saturate the solution at its boiling point. This is best accomplished by using sodium carbonate monohydrate in a quantity sufficiently large that a substantial part of it remains on the bottom of the vessel containing the bath. In this manner it is certain that the solution remains saturated at all times and temperatures. It is preferable to use distilled water in the bath as I find that this provides the best and most dependable coating. Tap water of normal purity may be used, although the quality of the coatings may then vary to some extent.

The term "magnesium" as herein used means any article made of pure magnesium or its commercial alloys.

The magnesium article to be coated is then immersed in the electrolyte while connected to the positive pole of a direct current source, the material thus being the anode. A commercial 110-125 volt direct current line may be used as the voltage source. During the operation of placing or immersing the magnesium article in the electrolyte, the current is preferably kept constant at whatever value the available equipment will furnish. It is preferable to use the highest current value possible consistent with the means provided for maintaining the electrolyte at or near its boiling temperature. For example, in my preferred practice the initial current value is approximately 100 amperes per square foot, although an initial current value range of 50-120 amperes per square foot may be used. If initial current value is substantially below 100 amperes the time required for completing the coating operation is increased. If necessary, a convenient means of regulating the initial current density is the use of a series resistance or of a constant current generator. If the magnesium article is immersed before application of the current, the time of coating may generally be increased.

Prior to the treatment, it is desirable, although not essential, to clean the surface of the magnesium of any dirt, grease or other undesired coating, by any of the well-known means. The electrolyte which I use is in itself an alkaline cleaner

and is capable of handling reasonably dirty objects without prior cleaning. Such procedure is generally undesirable, however, since the coatings produced may not be at times as perfect as they would be if the object had been previously cleaned, depending upon the material and extent of surface contamination. Also, in such case the electrolyte life will be somewhat impaired.

The coating begins to form as soon as the magnesium object is immersed in the electrolyte. This coating presents a relatively high electrical resistance when properly formed and thus causes a steady gradual decrease in the electric current which may flow at any given voltage. For example, using the voltage sufficient to provide an initial current density of approximately 100 amperes per square foot, if the coating formed is a proper one, the density will decrease to about 0.2 ampere per square foot within ten minutes, approaching ultimately some small fixed asymptotic value which varies with the purity of the alloy and is generally under 0.04 ampere per square foot for the usual commercial magnesium alloys used.

If the electrolyte is contaminated, or if the magnesium being treated contains flux inclusions, or segregation of alloying constituents, or if the surface is of low quality due to the presence of foreign elements on which no magnesium carbonate coating may be produced, the coating will be relatively porous or the surface will become etched rather than coated, so that the functioning of the coating as an electrical resistance is poor or erratic. Consequently, the current density will decrease for a short while during the early stages but will then tend to go up again. Where the magnesium is of poor quality, I have found it to be impossible to reduce the current density below  $\frac{1}{100}$  of its initial value, and at times, if the magnesium is of very poor quality, it is impossible to reduce the current density to below  $\frac{1}{10}$  of its initial value. Such objects are defective and should be discarded.

While, if the electrolyte is materially contaminated it will affect the decrease in current density, it is relatively easy to keep the bath free of any serious contamination and therefore it is a simple matter with the use of my invention to determine by measuring the current density from a given voltage just what are the characteristics of the coating and whether the magnesium object is faulty.

The coating produced by my invention is relatively non-porous as compared with the relatively porous coatings on magnesium resulting from electrochemical treatments heretofore attempted. This improved type of coating appears to be due, at least to some extent, to the fact that my coating has a greater volume than that occupied by the magnesium used in forming the coating, while the previously known coatings were relatively smaller in volume. My coating is relatively dense and is impermeable to the usual corrosion media to which magnesium is generally exposed.

Another factor contributing to the improved results of my method appears to be that my method produces an anhydrous magnesium carbonate coating which has no appreciable solubility in salt water saturated with  $\text{CO}_2$  or other normal corrosive, while the usual form of magnesium carbonate produced in aqueous media is relatively hydrated and has substantially the formula  $\text{MgCO}_3 \cdot 3\text{H}_2\text{O}$ .

The duration of the treatment determines the

thickness of the coating. I find sixty minutes to be adequate in most cases and after such period of treatment using a magnesium object of proper quality, the current density will have dropped to as low as 0.04 ampere per square foot. If such current density drop is not obtained, it denotes that the coating is not of the proper quality. The temperature of the bath should be maintained above  $50^\circ \text{C}$ , the optimum being  $90^\circ \text{C}$ .

While in my preferred example of bath I prescribe a saturated solution of sodium carbonate, I wish it understood that, in its broader aspects, my invention contemplates the use of any alkali carbonate capable of forming an anhydrous magnesium carbonate coating on magnesium and its alloys. For instance, ammonia carbonate may be used and other concentrations may be used. However, for any specific concentration an appropriate voltage and current schedule should be adopted, based upon the optimums which I have given hereinabove for a saturated sodium carbonate solution.

I claim:

1. The method of electrolytically forming a protective film on a magnesium object which comprises electrochemically treating the object, as an anode, in an electrolyte consisting of a substantially saturated solution of alkali carbonate while maintaining the solution about  $50^\circ \text{C}$ , the anodic treatment being continued until the current flow decreases to a relatively small value due to the electrical resistance of the resulting film.

2. The method of claim 1, wherein said alkali carbonate is sodium carbonate.

3. The method of claim 1, wherein said relatively small value of current flow is a current density below 0.2 amperes per square foot.

4. The method of electrolytically forming a protective film on a magnesium object which comprises electrochemically treating the object, as an anode, in an electrolyte consisting of a substantially saturated solution of sodium carbonate while maintaining the solution above about  $50^\circ \text{C}$ . with sodium carbonate in the solid phase in contact with said saturated solution, the anodic treatment being continued until the current flow decreases to a relatively small value due to the electrical resistance of the resulting protective film.

5. A method of treating magnesium articles to form a protective coating thereon which comprises subjecting the article, as an anode, to electrolytic treatment in an electrolyte consisting of a substantially saturated solution of alkali carbonate at a temperature above about  $50^\circ \text{C}$ . while imposing a voltage sufficient to maintain on the article a current density at the beginning of the formation of the coating of above 50 amperes per square foot and continuing the anodic action until the current flow decreases to a relatively small value, while determining the characteristics of the coating being formed by measuring the rate of decrease in current density caused by the formation of the coating and discarding the articles so treated which give erratic current density and which never attain coatings with predetermined electrical resistance.

6. The method of claim 5, in which said current above 50 amperes is a current density of between 50 and 120 amperes per square foot.

7. The method of claim 5, in which said alkali carbonate is sodium carbonate.

8. The method of claim 5, in which alkali carbonate in the solid phase is maintained in contact with the electrolyte used in the treatment.

9. The method of electrolytically forming a protective film on a magnesium object which comprises electrochemically treating the object, as an anode, in an electrolyte consisting of a substantially saturated solution of alkali carbonate while maintaining the solution above about 50° C., the anodic treatment being continued until there is formed on the article a protective film having greater volume than the volume of magnesium used in forming the coating and the current flow decreases to a relatively small value due to the electrical resistance of said film.

## REFERENCES CITED

The following references are of record in the file of this patent:

| UNITED STATES PATENTS |                |               |
|-----------------------|----------------|---------------|
| Number                | Name           | Date          |
| 1,117,240             | Presser        | Nov. 17, 1914 |
| 2,146,029             | Schimkus       | Feb. 7, 1939  |
| 10 2,197,611          | Fischer et al. | Apr. 16, 1940 |

## OTHER REFERENCES

Trans. Electrochem. Soc., vol. 68 (1935), pp. 533-547.

HERBERT WATERMAN.